

1

3,155,619

## COMPLEX LUBRICANT

Martin M. McCormick, Chicago, Ill., assignor to Sinclair Research, Inc., Wilmington, Del., a corporation of Delaware  
No Drawing. Filed Feb. 12, 1962, Ser. No. 172,783  
8 Claims. (Cl. 252—39)

This invention relates to a method for preparing high temperature lubricating compositions thickened to a grease consistency with a mixed salt-soap thickener. More particularly, the present invention relates to an improved method of manufacturing calcium acetate-fatty soap greases which are smooth and homogeneous and have a small spread between unworked and worked penetrations.

The use of mixed salt-soap thickeners as grease thickeners is well known in the art. In manufacture, these admixtures are generally subjected to a shearing force sufficient to disperse the soap in the base oil to form a grease structure. The shearing action involves the application of force in a plane and disperses the soap in an intimately orientated linear pattern. However, it has been found that if the shearing force is sufficient to improve the texture of greases in which the mole ratio of salt/soap is in excess of 3:1, the milling operation results in a grease having a very wide range between worked and unworked penetration even though the grease has a stable structure. This thixotropic spread is undesirable from the standpoint of slumpability into dispensing equipment and the limited ability of the grease to properly feed to surfaces requiring lubricating.

In brief, the present invention relates to a process for the preparation of smooth and homogeneous mixed salt-soap thickened greases having an acceptable low level of thixotropy and containing a molar ratio exceeding 3:1 of alkaline earth metal salt/soap type greases by employing a certain homogenizing sequence consisting essentially of an initial relatively high shear rate processing sufficient to obtain highly efficient and improved dispersion of the thickener followed by a lower shear rate operation sufficient to bring the worked and unworked penetrations of the greases in close proximity to one another. The term homogenizing is intended to include any method of subjecting the lubricant to shearing forces.

The mixed salt-soap thickeners of the invention can be formed by the neutralization with a metal base of a low molecular weight and a higher molecular weight carboxylic acid, for instance high molecular weight acids and intermediate molecular weight acids and combinations of the same. Therefore, the mixed salt-soap thickener may be formed from either a combination of (1) a low molecular weight acid and a high molecular weight acid, or (2) a low molecular weight acid and an intermediate molecular weight acid, or (3) a low molecular weight acid, an intermediate molecular weight acid and a high molecular weight acid, in which the mol ratio of low molecular weight acid to the other acids employed exceeds 3:1 and may be as high as 20:1 or more to be effectively utilized in the preparation of the present grease composition.

In the preparation of these mixed salt-soap thickeners, any suitable procedure may be used, for instance, a coneutralization, pre-forming or step-wise method. In the coneutralization method, a mixture of the low and high and/or intermediate molecular weight acids is neutralized with a suitable base, particularly the hydroxide and/or carbonate of the desired metals. This coneutralization step is generally carried out in a grease kettle "in situ," in the liquid menstruum to which the complex thickener is to be applied in actual use. For example, the mixed acids may be coneutralized in a portion or all of the lubricating oil forming the dispersant of

2

a grease to be thickened by the mixed salt-soap thickener. Coneutralization is possible in cases in which the salts have the same metal constituent, and the menstruum is inert under the conditions of saponification or neutralization. The coneutralized material may be heated to temperatures of about 250° to 500° F., preferably less than about 350° F., in order to dehydrate the product.

The mixed salt-soap thickener may also be prepared by separately preforming at least a portion of the high and/or intermediate molecular weight carboxylic acid salt, intimately mixing this salt with the low molecular weight salt and then heating, if necessary. This method is less desirable than coneutralization in situ and is perhaps most useful from a practical standpoint when different metals are employed in forming the different salts.

In the step-wise method the high molecular weight acid is melted in the base oil in the presence of the metal base and then the low and/or intermediate weight acids are added and the mixture is allowed to react at a temperature sufficient to render the grease substantially anhydrous.

The soap-forming fatty component contemplated in this invention are the saturated and unsaturated, naturally occurring or synthetic grease-making carboxylic fatty acids and their esters such as the naturally occurring or processed fats and oils which are in glyceride form, that are commonly known in the art and containing about 7 to 30 carbon atoms. In general, the higher fatty acids have from about 12 to 30 carbon atoms, preferably about 12 to 22 carbon atoms per molecule, and have saponification values of from about 270 to 170. The fatty acids normally used in the manufacture of conventional greases, particularly the saturated acids, are preferred. Suitable fatty acids include lauric, myristic acid, palmitic acid, stearic acid, the various hydroxy stearic acids, oleic acid, arachidic acid, behenic acid and the like. Naturally occurring fatty acids such as fish oil acids, tallow acids, which contain chiefly stearic acid, coconut oil acids, castor oil, etc. may also be utilized directly or after hydrogenation to decrease any undesirably high degree of unsaturation. Mixtures of these high molecular weight fatty acids, e.g., hydrogenated fish oil acids with oleic acid, in any proportions, are also operable, as are fractions obtained by distillation, extraction or crystallization.

The intermediate molecular weight monocarboxylic acids are those straight-chain, saturated fatty acids having from about 7 to 12 carbon atoms. Operable intermediate molecular weight carboxylic acids are exemplified by:

|                            | Mol. Weight | Sap. No.<br>(mgs. KOH/<br>gm.) |
|----------------------------|-------------|--------------------------------|
| Enanthic (heptanoic)-----  | 130         | 431                            |
| Caprylic (octanoic)-----   | 144         | 389                            |
| Pelargonic (nonanoic)----- | 158         | 354                            |
| Capric (decanoic)-----     | 172         | 326                            |

Caprylic, pelargonic, and capric acids are preferred. The intermediate molecular weight carboxylic acids of even carbon chain lengths are normally obtained by processing from naturally-occurring materials such as coconut oils.

Pelargonic acid is obtained as a by-product in the production of azelaic acid by the ozonolysis of oleic acid.

Suitable low molecular weight acids include saturated and unsaturated aliphatic monocarboxylic acids having about 1 to 4 carbon atoms, such as formic, acetic, propionic, furoic, acrylic and similar acids including their hydroxy derivatives, such as lactic acid. Acetic acid is especially preferred. The acetic acid can be glacial acetic acid or an aqueous solution of acetic acid. The concentration of acid in the solution often varies from about 60 to 99.9 weight percent, and is preferably about 80 weight percent. The use of a substituted acetic acid is

not excluded, where such modification may be desirable. For example, chloro-acetic acid may be used to modify the structure of a grease made in accordance with the invention.

The metal component of the thickener system of the invention is used in a form which can combine chemically with carboxylic acids to form salts or soaps. Ordinarily the metal hydroxide is used. The choice of metal component depends to a certain extent on the use to which the multiple salt and soap thickener of the invention is to be put. The alkaline earth metal hydroxides or carbonates such as those of calcium, barium and strontium are useful for many purposes of the invention. Calcium hydroxide or hydrated lime is especially preferred.

The lubrication oil may be either a mineral base lubricating oil or various synthetic oils. Mineral base lubricating oils ranging in viscosity from about 30-1000 SSU at 100° F. are preferably employed as the liquid phase of the grease compositions of the invention. These naturally occurring mineral lubricating oils may be derived from any petroleum crude source, whether paraffinic or naphthenic in type, and may be refined by any of the known refining techniques of the petroleum industry.

The invention is not limited, however, to the use of mineral base oils, since various synthetic oils having at least 30 Saybolt Universal viscosity at 100° F. may also be used as part or all of the liquid phase of the grease. Examples of operable synthetic lubricating oils include ether alcohols, such as those corresponding to the general formula



wherein R is an alkyl group, e.g., butyl, n is an integer from 2 to 5, and x is an integer from 1 to 40; esters of monobasic carboxylic acids, totalling 8 to 80 carbon atoms, such as those of C<sub>4</sub> to C<sub>18</sub> aliphatic acids with C<sub>4</sub> to C<sub>18</sub> aliphatic alcohols, the C<sub>4</sub> to C<sub>18</sub> radicals including the butyl, isobutyl, hexyl, octyl, iso-octyl, 2-ethyl hexyl, nonyl, decyl, lauryl, stearyl and similar radicals; diesters of dibasic acids, such as adipic or sebacic acid with monohydric alcohols, such as hexyl, octyl, 2-ethyl hexyl or higher alcohols; esters of polyethylene glycols with C<sub>8</sub> to C<sub>18</sub> branched-chain carboxylic acids; complex esters of polybasic carboxylic acids, polyhydric alcohols, and monobasic acids and/or monohydric alcohols, such as the glycol-centered or dibasic acid-centered complex esters; phosphoric acid esters or thioesters of aliphatic alcohols or mercaptans of up to about 18 carbon atoms; halocarbon oils, such as the polymers of chlorofluoro alkynes like chlorotrifluoroethylene; organo-siloxanes; sulfite esters, organic carbonates; mercaptals; formals, etc.

In preparing the lubricating grease composition of this invention, about 50 to 95 weight percent of lubricating oil and from about 5 to 50 weight percent of the mixed salt-soap thickener may be used. A preferred range is from about 10 to 30 weight percent of the mixed salt-soap thickener, based on the weight of the total composition. This mixed salt-soap thickener, in turn, can be prepared by using 1 mole of the high and/or intermediate molecular weight acid with about 3 to 15 or 20 or more mols, preferably 5 to 12 mols of the low molecular weight acid with stoichiometric amounts of the metal base sufficient to react with the acids and other saponifiable components of the thickener system.

The greases may also contain various additives of the usual type such as corrosion inhibitors, oxidation inhibitors, anti-wear agents, extreme pressure agents, etc. The additive may be added either before or during the cooling down process. They are preferably added while the temperature of the grease is between about 300° F. and about 180° F.

In general, the lubricating grease compositions can be made in any way desired, for instance by mixing together the desired amount of mineral or synthetic lubricat-

ing oil, the base and the high molecular weight carboxylic acid. The acetic acid and the intermediate molecular weight carboxylic acid, if one is employed, are then added to the mixture, and allowed to react without further external heating. When temperature of the reaction starts to subside, external heating is then applied and is continued until the temperature is within the range of about 250-500° F. until the water content is below about 0.5 weight percent rendering the grease substantially anhydrous. The exact temperature range which may be used varies from one process to another depending upon different procedural steps fully understood by those skilled in the art. When the maximum temperature desired is reached, heating may be discontinued and the grease batch is cooled to about 250° F. Any of the conventional anti-oxidant additives, such as phenyl alpha naphthylamine, may be added at this time, and the grease is further cooled to below about 200° F. The resulting grease composition is then homogenized by passing the grease through a suitable high shear rate milling device, such as for example, a Charlotte Colloid Mill, Mantin-Gaulin Homogenizer, Morehouse Mill, Cornell Deaerator and Turbinizer (Lancaster Dispenser) which have shearing rates in the range of about 5000 to 500,000 reciprocal seconds sufficient to complete the mixing operation in a short period of time and obtain smooth, buttery-texture grease. Before homogenization many of these greases have in addition to a rough texture a softer un-worked than worked consistency. The homogenizing operation results in a large amount of hardening of the greases on the basis of both worked and unworked penetration. Also, it has been found that when a mixed salt-soap thickened grease having a salt/soap ratio in excess of 3:1, is homogenized under sufficient shear rate to improve the grease's texture, i.e. about 5000 to 500,000 reciprocal seconds, there will result a large spread between the unworked and worked consistency amounting to more than an NLGI grade range. As mentioned above, this excessive spread is undesirable from the standpoint of slippability and its effectiveness to be properly fed to surfaces requiring lubrication. However, this undesirable penetration spread is essentially eliminated by the high shear-low shear homogenizing treatment of the present invention.

The consistency of the grease is measured in terms of penetration at 77° F. using an ASTM conical type penetrometer, for instance, ASTM method D-217-60-T. The grease is mechanically worked in an ASTM grease worker, which consists essentially of a piston and cylinder assembly wherein the piston is a disk having many relatively small perforations. The cylinder is charged with grease, and the piston reciprocated, thus rapidly forcing the grease through the perforations. This penetration is generally measured before working and after 60 and 10,000 or 100,000 full double strokes.

In the preparation of calcium acetate/soap greases having a molar ratio in excess of 3:1, a suitable range for shearing is below about 225° F., preferably below about 200° F. The initial homogenization applied to the calcium acetate/soap greases is of sufficient shear rate to obtain highly efficient and improved dispersion of the thickener. This shearing on all or a substantial or major portion of the grease imparts to the grease a consistency spread between unworked and worked penetrations at 77° F. in the range of about 25 to 75 mm./10, usually about 30 to 60 mm./10. The second homogenization is again conducted on all or a substantial or major portion of the grease and is of low shear and brings the unworked and worked penetrations of the greases to a range of about 0-15 mm./10, preferably about 0 to 10 mm./10. In terms of shearing force the initial homogenization should be in the range of about 5,000 to 500,000 reciprocal seconds, preferably from about 10,000 to 200,000 reciprocal seconds. The low shearing rate should be in the range between about 1 to 500 reciprocal seconds, preferably

from about 1 to 300 reciprocal seconds. For instance, in the examples described below, the high shear rate used is about 75,000 reciprocal seconds and the low shear about 45 reciprocal seconds.

In the process of the present invention it should be understood that the high shear rate treatment is not necessarily initial or the low shear rate second, it is, however, essential that the low shear treatment follows the high shear as a final step in the processing sequence. For instance, in the examples described below the grease is continuously passed from a low shear rate zone, the mixing kettle, through a high shear rate device, such as a Colloid Mill, and passed either back to the low shear rate mixing zone or another suitable low shear rate device for a period of time sufficient to obtain the above-mentioned desired results as the final step in the processing sequence.

The present invention will be more fully understood by reference to the following specific examples which illustrate the processing method of the present invention.

#### EXAMPLE I

A commercial calcium acetate/mixed fatty soap grease having a molar ratio of calcium salt/soap of 6:1 was prepared having the following composition:

|                                   | Weight, lbs. | 20 |
|-----------------------------------|--------------|----|
| Glacial acetic acid               | 909          |    |
| Vegetable fatty acid <sup>1</sup> | 362          |    |
| Tallow fatty acid                 | 120          |    |
| Hydrogenated castor oil           | 120          |    |
| Hydrated lime                     | 680          | 30 |
| 430 SUS/100° F. M.C. neutral      | 6440         |    |
| Age Rite Resin D                  | 42           |    |

<sup>1</sup> Straight chain fatty acid having the following characteristics:

|                          |     |    |
|--------------------------|-----|----|
| Acid No.                 | 240 | 35 |
| Saponification No.       | 240 |    |
| Iodine value             | 62  |    |
| Average molecular weight | 233 |    |

The grease was separated into four samples and tested in terms of penetration at 77° F. using as ASTM conical type penetrometer before and after certain homogenizing procedures. The results are tabulated in Table I.

Table I

|                              |               |                   |                                            |                           |                                                   |                 |
|------------------------------|---------------|-------------------|--------------------------------------------|---------------------------|---------------------------------------------------|-----------------|
| Calcium Acetate, Wt. percent | 15.0          |                   |                                            |                           | 14.2                                              |                 |
| Calcium Soap, Wt. percent    | 8.2           |                   |                                            |                           | 7.8                                               |                 |
| Moisture, Wt. percent        |               |                   |                                            |                           | 0.3                                               |                 |
| Free CaO, Wt. percent        |               |                   |                                            |                           | 0.29                                              |                 |
| Sample No.                   | 90            | 91                | 92                                         | 92A                       | 93*                                               | 95              |
|                              | Kettle Sample | Cornell Daeerator | Charlotte Colloid Mill & Cornell Daeerator | Recycle thru Colloid Mill | Recycle to Kettle thru Colloid Mill and Daeerator | Oil added to 93 |
| ASTM Penetrations, mm./10:   |               |                   |                                            |                           |                                                   |                 |
| Unworked                     | 318           | 237               | 224                                        | 203                       | 250                                               | 283             |
| Worked (60 strokes)          | 294           | 270               | 261                                        | 228                       | 248                                               | 280             |
| Texture                      | Rough         | Smooth            | Smooth                                     | Smooth                    | Smooth                                            | Smooth          |

\*Recycled around kettle through colloid mill and deaerator for 45 minutes at 0.005" clearance at an inlet temperature of 180° F. and a rate of 190 lbs./min.

It is to be noted that the Kettle Sample (Sample 90) exhibitions a rough texture and softer consistency unworked than worked. When the grease is homogenized to obtain a smooth texture at high shear (Samples 91 and 92), there results a large spread between the unworked and worked penetrations. Even after a second pass through the high shear homogenizer, the Colloid Mill (Sample 92A), there still exists a large spread between unworked and worked penetrations. Also, after a high shear homogenizing the grease has a harder consistency unworked than it does worked. However, by recycling the grease through the homogenizer and back to the kettle

(low shear homogenizing) for 45 minutes, which corresponds to a complete turnover of the batch, the spread between the unworked and worked penetration is very small while the grease still retains a smooth texture (Sample 93).

#### EXAMPLE II

An 8:51 molar ratio calcium acetate/mixed fatty soap grease having the following composition was prepared.

Component, lbs:

|    |                              |       |
|----|------------------------------|-------|
| 10 | Glacial acetic acid          | 60.5  |
|    | Vegetable fatty acid         | 18.25 |
|    | Tallow fatty acid            | 6.2   |
|    | Hydrogenated castor oil      | 6.2   |
| 15 | Hydrated lime                | 43.0  |
|    | 430 SUS/100° F. M.C. neutral | 410.0 |

The grease was treated as indicated in Table II.

Table II

|    |                              |                          |                               |                                          |
|----|------------------------------|--------------------------|-------------------------------|------------------------------------------|
| 20 | Calcium Acetate, Wt. Percent | 15.2                     |                               |                                          |
|    | Calcium Soap, Wt. Percent    | 6.3                      |                               |                                          |
|    | Moisture, Wt. Percent        | 0.6                      |                               |                                          |
|    | Free CaO, Wt. Percent        | 0.26                     |                               |                                          |
| 25 | Sample No.                   | 96                       | 96A                           | 96B*                                     |
|    |                              | Kettle Sample (Unmilled) | Colloid Milled (Once through) | Recycle Colloid Milled around the kettle |
| 30 | ASTM Penetrations, mm./10:   |                          |                               |                                          |
|    | Unworked                     | 306                      | 233                           | 297                                      |
|    | Worked (60 Strokes)          | 319                      | 289                           | 292                                      |

\* Recycled 25 minutes through colloid mill (Charlotte No. 3) at 0.005" clearance with an inlet temperature of 170° F. and an outlet temperature of 175° F. at a rate of 18 lbs./minute. The grease is then mixed with pump recycle by-passing the colloid mill for another 25 minutes. The samples were recovered at 168° F.

EXAMPLE III  
A 6:1 molar ratio of calcium acetate/mixed fatty

It is to be noted that the Kettle Sample (Sample 90) exhibitions a rough texture and softer consistency unworked than worked. When the grease is homogenized to obtain a smooth texture at high shear (Samples 91 and 92), there results a large spread between the unworked and worked penetrations. Even after a second pass through the high shear homogenizer, the Colloid Mill (Sample 92A), there still exists a large spread between unworked and worked penetrations. Also, after a high shear homogenizing the grease has a harder consistency unworked than it does worked. However, by recycling the grease through the homogenizer and back to the kettle

soap grease having the following composition was prepared.

Components, lbs.:

|    |                              |       |
|----|------------------------------|-------|
| 70 | Glacial acetic acid          | 48.0  |
|    | Hydrogenated coconut acid    | 12.8  |
|    | Vegetable fatty acid         | 12.8  |
|    | Hydrogenated castor oil      | 6.4   |
|    | Hydrated lime                | 35.0  |
|    | 430 SUS/100° F. M.C. neutral | 340.0 |

The grease was treated as shown in Table III.

7  
Table III

|                                             |                          |                                      |
|---------------------------------------------|--------------------------|--------------------------------------|
| Calcium Acetate, Wt. Percent.....           | 14.4                     |                                      |
| Calcium Soap, Wt. Percent.....              | 8.2                      |                                      |
| Moisture, Wt. Percent.....                  | 0.2                      |                                      |
| Free CaO, Wt. Percent.....                  | 0.12                     |                                      |
| Sample No.....                              | 97                       | 97A                                  |
|                                             | Kettle sample (unmilled) | Colloid Milled (once through)        |
|                                             |                          | Recycle Colloid milled around Kettle |
| ASTM Penetrations, mm./10:<br>Unworked..... | 295                      | 209                                  |
| Worked (60 Strokes).....                    | 298                      | 260                                  |

\* Recycled 20 minutes around kettle through colloid mill at 0.005" clearance with an inlet temperature of 185° F. and an outlet temperature of 194° F. at a rate of 20 lbs./minute. The grease is then mixed with pump, recycle by passing the mill for an additional 30 minutes. The samples were drawn at 176° F.

## EXAMPLE IV

Two batches of 7:1 molar ratio calcium acetate/mixed fatty soap greases having the following compositions were prepared.

| Components, lbs.                  | Sample No. 98 | Sample No. 99 |
|-----------------------------------|---------------|---------------|
| Glacial Acetic Acid.....          | 48.1          | 48.25         |
| Vegetable Fatty Acid.....         | 19.25         | 25.75         |
| Hydrogenated Castor Oil.....      | 12.82         | 6.44          |
| Hydrated Lime.....                | 34.75         | 35.0          |
| 430 SUS/100° F. M.C. Neutral..... | 350.0         | 365.0         |

The greases were treated as shown in Table IV.

Table IV

|                                     |                 |                |                |                 |
|-------------------------------------|-----------------|----------------|----------------|-----------------|
| Calcium Acetate, Wt. Percent.....   | 14.1            |                | 13.7           |                 |
| Calcium Soap, Wt. Percent.....      | 7.7             |                | 7.5            |                 |
| Moisture, Wt. Percent.....          | 0.6             |                | 0.6            |                 |
| Free CaO, Wt. Percent.....          | 0.08            |                | 0.07           |                 |
| Sample No. 801P.....                | 98              | 98A            | 98B*           | 99              |
|                                     | Unmilled grease | Colloid milled | Recycle milled | Unmilled grease |
|                                     |                 |                |                | Colloid milled  |
| ASTM Penetrations:<br>Unworked..... | 312             | 192            | 267            | 319             |
| Worked (60 Strokes).....            | 277             | 239            | 264            | 289             |

\*Recycle Colloid Milling Conditions:

|                                                                                       |     |     |
|---------------------------------------------------------------------------------------|-----|-----|
| No. 3 Charlotte, 0.005" Clearance 20 lbs./minute rate, 20 minutes:<br>Inlet, ° F..... | 180 |     |
| Outlet, ° F.....                                                                      | 191 | 175 |
| Additional Kettle Mixing, Minutes.....                                                | 30  | 187 |

## EXAMPLE V

A 5.5:1 molar ratio calcium acetate/mixed fatty soap grease having the following composition was prepared.

| Components, lbs.:                        |       |
|------------------------------------------|-------|
| Glacial acetic acid.....                 | 48.0  |
| Emery coconut acid (chiefly lauric)..... | 25.6  |
| Hydrogenated castor oil.....             | 6.4   |
| Hydrated lime.....                       | 35.25 |
| 430 SUS/100° F. M.C. neutral.....        | 320.0 |

8  
Table V

|                                             |                 |                               |                                          |
|---------------------------------------------|-----------------|-------------------------------|------------------------------------------|
| Calcium Acetate, Wt. percent.....           | 15.0            |                               |                                          |
| Calcium Soap, Wt. percent.....              | 8.2             |                               |                                          |
| Moisture, Wt. percent.....                  | 0.15            |                               |                                          |
| Free CaO, Wt. percent.....                  | 0.01            |                               |                                          |
| Sample No.....                              | 100             | 100A                          | 100B                                     |
|                                             | Unmilled grease | Colloid Milled (once through) | Sample 100A colloid milled a second time |
|                                             |                 |                               | Recycle milled                           |
| ASTM Penetrations, mm./10:<br>Unworked..... | 298             | 199                           | 183                                      |
| Worked (60 strokes).....                    | 286             | 253                           | 230                                      |

\*Recycle Colloid Milling Conditions:

No. 3 Charlotte, 0.005" Clearance 25 lbs/min. rate, 15 minutes—  
Inlet Temperature, ° F..... 181  
Outlet Temperature, ° F..... 199  
Additional Kettle Mixing, minutes..... 30

In Table V, it is to be noted that a large spread between unworked and worked penetrations still exists even after a second pass through the high shear homogenizer, the Colloid Mill (Sample No. 100B). However, when a low shear processing treatment followed the initial high shear rate homogenizing, there resulted a small spread between the unworked and worked consistencies (Sample No. 100C).

It can be readily seen in Examples I through V that the smooth texture obtained in the high shear homogenization was retained following the low shear homogenization step while the spread between the unworked and worked consistencies was reduced.

It is claimed:

1. A process for the preparation of a lubricating grease consisting essentially of an oil of lubricating viscosity

and a grease thickening amount of a mixed salt-soap thickener consisting essentially of an alkaline earth metal salt of acetic acid and an alkaline earth metal soap of a higher molecular weight carboxylic acid of about 7 to 30 carbon atoms, wherein said salt of acetic acid and said soap of said higher molecular weight carboxylic acid are in a molar ratio of about 3:1 to 20:1, the improvement which consists essentially of shearing said grease at a rate in the range of about 5,000 to 500,000 reciprocal seconds sufficient to obtain a dispersion of the thickener, followed

by shearing said grease at a rate in the range of about 1 to 500 reciprocal seconds to obtain a final grease composition.

2. The process of claim 1 wherein the higher molecular weight carboxylic acid is selected from the group consisting of carboxylic acids containing about 12 to 30 carbon atoms, carboxylic acids containing about 7 to 12 carbon atoms and combinations of the same.

3. The process of claim 1 wherein the initial homogenization of the mixed salt-soap thickened grease is conducted in the range of about 10,000 to 200,000 reciprocal seconds.

4. The process of claim 1 wherein the second homogenization of the mixed salt-soap thickened grease is conducted in the range of about 1 to 300 reciprocal seconds.

5. A process for the preparation of a lubricating grease consisting essentially of an oil of lubricating viscosity in amounts of about 50 to 95% of final composition and about 5 to 50 weight percent of a mixed salt-soap thickener consisting essentially of an alkaline earth metal salt of acetic acid and an alkaline earth metal soap of a higher molecular weight carboxylic acid of about 7 to 30 carbon atoms wherein said salt of acetic acid and said soap of a higher molecular weight acid are in a molar ratio of about 3:1 to 20:1, the improvement which consists essentially of shearing said grease at a rate in the range of about 5000 to

500,000 reciprocal seconds, sufficient to obtain a dispersion of the thickener and a spread between unworked and 60 stroke worked penetration of about 25 to 75 mm./10 followed by shearing said grease at a rate in the range of about 1 to 500 reciprocal seconds to obtain a grease composition having a maximum spread between unworked and 60 stroke worked penetration of about 15 mm./10.

6. The process of claim 5 wherein the higher molecular weight carboxylic acid is selected from the group consisting of carboxylic acids containing about 12 to 30 carbon atoms, carboxylic acids containing about 7 to 12 carbon atoms and combinations of the same.

7. The process of claim 5 wherein the initial homogenization of the mixed salt-soap thickened grease is conducted in the range of about 10,000 to 200,000 reciprocal seconds.

8. The process of claim 5 wherein the second homogenization of the mixed salt-soap thickened grease is conducted in the range of about 1 to 300 reciprocal seconds.

References Cited in the file of this patent

UNITED STATES PATENTS

|    |           |                        |               |
|----|-----------|------------------------|---------------|
| 25 | 2,850,458 | Beerbower et al. ----- | Sept. 2, 1958 |
|    | 2,973,321 | Morway et al. -----    | Feb. 28, 1961 |
|    | 2,976,242 | Morway -----           | Mar. 21, 1961 |